

## UNITED STATES PATENT OFFICE.

JOHN MORCZEWSKI, OF SOUTH BEND, INDIANA, ASSIGNOR OF ONE-THIRD TO ANDREW A. KEKKO, OF SOUTH BEND, INDIANA.

## CANDLE.

No Drawing.

Application filed December 6, 1926. Serial No. 153,043.

This invention relates to improvements in compositions of matter and more particularly to a candle composition,—one object of the invention being to provide a candle which shall be composed of such intermixed ingredients that it will consume substantially as fast as it melts during burning and thus obviate "dripping".

A further object is to provide a composition for a candle which shall be well adapted to contain perfume and effectually emit the fumes thereof during the burning of the candle.

With these and other objects in view, the invention consists in certain intermixed ingredients for a candle as hereinafter set forth and pointed out in the claim.

My improved composition comprises the following ingredients in the proportions substantially as specified:

|                    | Per cent. |
|--------------------|-----------|
| Oil of wintergreen | 1         |
| Kerosene           | 1         |
| Aqua ammonia       | 8         |
| 25 Glycerine       | 1         |
| Banana oil         | 2         |
| Paraffin           | 87        |

and with these ingredients a suitable perfume, such as any commercial cologne or fragrant liquid extract in any desired proportion will preferably be incorporated. I have found from experience that a candle composition such as above defined, is particularly well adapted to receive perfume thoroughly distributed and to insure the uniform emission of the fumes during the burning of the candle.

In preparing the composition, I prefer first to make a solution of the wintergreen

oil, kerosene, aqua ammonia, glycerine and 40 banana oil together with the perfume and then after melting the paraffin, to pour said solution into such melted paraffin and thoroughly mix it with the latter by stirring or in any other suitable manner. The composition will then be ready to be molded or otherwise formed into desired shape for use as candles.

I have demonstrated that in actual use the candle will consume approximately as fast 50 as the material melts and that a cup will form around the wick, which cup contains semi-melted material during the burning of the candle, but that melted material will not find its way to the exterior wall of the candle and therefore "dripping" will be obviated.

The glycerine aids in mixing the other ingredients smoothly with the paraffine while the ammonia imparts hardness to the cooling candle compound and the wintergreen and banana oil tend to counteract the strong scent of the ammonia and kerosene, so that less cologne, if it be used, will be more satisfactory than would otherwise be the case.

Having fully described my invention what I claim as new and desire to secure by Letters-Patent, is:

A candle composition consisting of paraffine 87 per cent and the product of an admixture of wintergreen oil one per cent, kerosene one per cent, aqua ammonia eight per cent, glycerine one per cent and banana oil two per cent, in the proportions substantially as specified.

In testimony whereof, I have signed this specification.

JOHN MORCZEWSKI.